

Patented Aug. 28, 1923.

1,466,301

# UNITED STATES PATENT OFFICE.

JOHN T. JONES, OF PITTSBURGH, PENNSYLVANIA, ASSIGNOR TO HOWELLS METAL-  
LURGICAL COMPANY, OF PITTSBURGH, PENNSYLVANIA, A CORPORATION OF  
PENNSYLVANIA.

## PROCESS FOR PRODUCING STEEL.

No Drawing.

Application filed July 19, 1918. Serial No. 245,656.

To all whom it may concern:

Be it known that I, JOHN T. JONES, a citizen of the United States, and a resident of Pittsburgh, in the county of Allegheny and 5 State of Pennsylvania, have invented certain new and useful Improvements in Processes for Producing Steel, of which the following is a specification.

My invention relates to improvements in 10 processes for producing steel and it consists in the steps hereinafter set forth.

The invention relates more particularly to a process for producing high grade steel, such as tool steel, armor plate, and other 15 steels which require a certain degree of hardness to render them capable of being used for the particular purposes for which they are designed.

In making steel by the Bessemer or the 20 open hearth process, it has heretofore been customary to make use of other metals, such as manganese or silicon in one form or another for the purpose of taking up excess oxygen and also for the purpose of recarburizing. The form in which these metals are used is generally that of an alloy and the 25 alloys are relatively expensive, thus adding to the cost of the finished product.

The primary object of my invention is to 30 provide a process by means of which a cheap deoxidizing and recarburizing agent may be used to obtain a product of the highest grade steel.

A further object of the invention is to 35 provide a process by means of which iron which has already been made, may be so hardened that its nature is changed and it becomes in fact a high grade steel.

A further object of the invention is to 40 provide a process whereby iron of a fibrous nature, such as wrought iron, may be treated so that the outer surface may be rendered extremely hard, the hardness decreasing toward the center so as to provide a central 45 portion of tough fibrous material having a hard exterior.

Other objects and advantages will appear 50 in the following specification and the novel features of the invention will be particularly pointed out in the appended claims.

In carrying out my process I make use of one of the cheapest forms of pig iron, as for instance #6 charcoal pig iron. This pig iron contains from four to six per cent of

carbon combined with the iron, as distinguished from other forms of pig iron in which the carbon may exist as in the graphitic state. It may be made by taking iron ore, as for instance from the Menominee range, which contains approximately forty 55 per cent of iron and .002 per cent of phosphorus. When charcoal or coke is used to make this pig iron it produces a pig having substantially .01 per cent of phosphorus. This pig iron melts at a temperature of from 60 1800° F. to 2000° F. The above is given as illustration only, since any form of pig iron having its carbon in combined form would suffice for the purposes of this invention, although the particular pig iron mentioned 65 i. e. #6 charcoal pig, I find is best suited to the purpose.

From 500 to 2000 pounds of the molten pig is added to the steel bath which comprises the charge of a Bessemer converter or 70 an open hearth furnace, depending upon the size of the converter or furnace used. The molten pig iron has the effect of taking up the excess oxygen or the "overblow" in the Bessemer converter, and furthermore, recarburizes the charge so that the steel produced is of the highest grade. This obviates the necessity of the use of ferromanganese or spiegeleisen. The reduction in the cost of 75 the operation is considerable when it is taken into account that the ferromanganese costs about \$300 per ton as against \$20 for #6 pig iron, other conditions being equal.

The product formed is an exceedingly high grade steel. The presence of the pig 80 iron removes the excess oxygen in the metal, rendering it free from blow holes and other defects.

The use of the pig iron in hardening, also produces high grade products at a relatively 85 low cost. The piece to be hardened is raised to the same temperature as the melting point of the pig iron. It is then immersed in the melted pig iron, or that portion which is designed to be hardened is so immersed, for 90 a short time. This time varies in accordance with the different implements or objects to be hardened. After the object is thus treated, it is plunged into cold water 95 and is immediately available for use.

It is desirable in many instances to provide devices or objects having hard wear-resisting exteriors and softer interiors. A 100

car wheel for instance, may be made with a tough central portion and the rim of the wheel may be hardened by my improved process, by supporting the wheel on an arbor 5 and turning it to bring the rim into contact with the molten pig iron. The depth to which the tread of the wheel is hardened depends upon the depth to which it is immersed in the melted pig iron. A shaft 10 may be hardened in the same way, or any similar article.

In each instance a new product is formed. In the case of the Bessemer furnace or the open hearth furnace, the pig iron accomplishes what is usually accomplished by the more expensive deoxidizers and recarburizers. When articles are hardened by this process the composition of the article is actually changed since more carbon is added 20 and a certain proportion of the oxygen is taken up. This process differs therefore, from those hardening processes in which the iron or steel is merely chilled. As a matter of fact, when fibrous irons, such as wrought 25 iron, are used, that portion of the article which is immersed in the melted pig iron is changed to steel of the highest quality.

It will be seen from the description given above that the process of producing a high 30 grade steel may be economically carried out due to the fact that the deoxidizing and recarburizing agents may be had at a relatively low cost.

I claim:—

35 1. The process which comprises treating a surface of an article made of iron or steel

with a material for deoxidizing and carburizing said surface, said material comprising molten pig iron containing carbon in a combined state. 40

2. The process which comprises treating a surface of an article made of iron or steel with white charcoal pig iron to carburize said surface.

3. The herein described steps in the process 45 of producing a high grade steel, which consists in adding to a molten charge of iron or steel a material for deoxidizing and carburizing, said material comprising a pig iron containing carbon in a combined state. 50

4. The herein described process of producing a high grade steel which consists in adding to a molten charge of iron or steel, a pig iron containing carbon in a combined state, and having substantially .01 per 55 cent of phosphorus the carbon of the pig iron deoxidizing and carburizing the charge.

5. The herein described steps in the process of producing high grade steel, which consists in adding to a molten charge of iron or steel, white charcoal pig iron which deoxidizes and carburizes the charge. 60

6. The herein described process of producing a high grade steel which consists in adding to a molten charge of iron or steel white charcoal pig iron having substantially .01 per cent of phosphorus, said pig iron having a melting temperature of from 1800° F. to 2000° F. the carbon of the pig iron deoxidizing and carburizing the charge. 65

JOHN T. JONES.